

Aug. 25, 1931.

H. B. KIPPER

1,820,276

PROCESS OF WOOD DIGESTION

Filed Feb. 15, 1926



Fig. 1.



Fig. 2.

Inventor  
Herman B. Kipper  
By  
Frank E. Liverance, Jr.  
Attorney.

Patented Aug. 25, 1931

1,820,276

# UNITED STATES PATENT OFFICE

HERMAN B. KIPPER, OF MUSKEGON, MICHIGAN

## PROCESS OF WOOD DIGESTION

Application filed February 15, 1926. Serial No. 88,420.

This invention relates to a process of digesting wood to pulp. It is a primary object and purpose of the present invention to procure the proper digestion of wood to pulp much more rapidly than heretofore, the time of digestion being very greatly reduced so that a greatly increased production of pulp is obtained. Essentially, the process consists in the simultaneous grinding and digesting of the wood to pulp with a continual agitating of the material so that the digestion liquor is at all times intimately in contact with all portions of the material being digested.

An understanding of the invention may be had from the following description taken in connection with the accompanying drawings, in which,

Fig. 1 is a longitudinal vertical section through one form of apparatus which may be used to carry out the process, and,

Fig. 2 is a transverse vertical section substantially on the plane of line 2—2 of Fig. 1.

In the construction of the apparatus a cylindrical container 1 is provided having ends 2 closing the same. At one end of the container and at its upper side, an inlet at 3 is made for the admission of the wood chips and digestion liquor into the container. The inlet is adapted to be closed by a bolted and gasketed cover 3a. The finished pulp and the spent or black liquor are withdrawn from the container through an outlet pipe 4 having a suitable valve which may be opened or closed by manual operation of the hand wheel 5. This outlet pipe is at the lower side and opposite end of the apparatus. Steam is admitted to the interior of the container through a pipe 6 and the pressure within the container is made known by gauge 7 of conventional construction.

Through each of the ends 2 a sleeve 8 is passed, the same being rotatably mounted and a suitable steam tight packing or stuffing box construction 9 is applied to each sleeve to prevent the escape of steam or other gaseous materials around the outside of said sleeves. At the inner end of each sleeve a plate 10 is secured having a diameter somewhat less than the interior diameter of the cylinder 1 and a plurality of scraper bars 11 are dis-

posed horizontally and at spaced apart intervals between and around the plates 10. These bars are reinforced between their ends by rings 12 located at and attached to their inner sides. The bars which are moved slowly over the inner surfaces of the container 1 are for the purpose of scraping the pulp from the said surfaces should the same deposit and build up on said surfaces. The use of said bars while very desirable in the apparatus is not absolutely essential.

A shaft 13 extends through said sleeves 8 the full length of the container and beyond the outer end of each sleeve, there being additional suitable packings indicated at 14 applied to the outer ends of the sleeves to prevent escape of gases around the shaft and between the shaft and the inner sides of the sleeves. Shaft 13 is rotatably supported at each end in suitable bearings at the upper ends of posts 15, and at one end the shaft is extended a distance beyond its adjacent post and is equipped with an additional bearing at the upper end of a post 15a. On said shaft within the container and at spaced apart intervals are fixed a plurality of spiders 16 having outwardly extending spaced apart arms which carry the beater or grinding bars 17 which may be rigidly attached to the ends of said arms, as shown, or may be mounted, as shown in my pending application, Ser. No. 739,040, filed September 22, 1924, so as to obtain a more complete grinding and beating action.

On the shaft 13 between the posts 15 and 15a a pulley 18 is mounted which may be driven by a belt 19 from any suitable source of power. The shaft 13 with its attached beating and grinding bars 17 is rotated at high speed. Near the end of shaft 13 a smaller pulley 20 is fixed which, through a belt 21, drives another pulley 22 fixed to a shaft 23. The shaft 23 is associated with a reduction gearing of any suitable form housed within the housing 24 so as to drive the shaft 25 at slow speed. Shaft 25 extends the full length of the apparatus and is mounted in suitable bearings in supports 26. The shaft 25 is equipped with sprocket wheels 27 in the same plane with which are large

sprocket wheels 28 fixed to the sleeves 8. The wheels 28 are driven from the wheels 27 by chains 29, it being evident that the sleeves 8 and the parts connected therewith move very slowly compared to the movement of the shaft 13 and the parts attached thereto.

The material which is introduced through the inlet 3 consists of wood chips and the digestion liquor. The digestion liquor is of well known composition including approximately 58% caustic soda, 27% sodium sulfide and 15% sodium carbonate dissolved in water, there being 1.37 grams of the solids named to each liter of digestion liquid.

15 Steam at one hundred pounds pressure is introduced into the container 1 through the pipe 6. The rapid rotation of the bars 17 not only continually stirs and agitates the material but the bars striking the same rapidly beat it to a pulp and the digestion liquor permeates the entire mass and is brought intimately into contact with all of the particles of wood chips as they are ground and beaten up by the apparatus. There is a tendency for 20 the pulp to adhere to the inner surface of the cylinder 1 and build up thereon to a certain depth and this is guarded against by the scraper bars 11 which continually remove any deposit which attempts to adhere to the walls 25 of the container.

The principal advantage of the process outlined consists in the rapid digestion of the wood, from one half to three fourths of an hour only being required to thoroughly 30 digest and reduce to pulp a batch of material placed in the apparatus as against two and one half to three hours required by the regular Kraft digestion process. The digested pulp with the spent or so-called "black liquor" is discharged through the outlet at 4, the black liquor being recovered from the 35 pulp and reclaimed for future use.

This process is very practical and its commercial utility and advantages are evident 40 from the greatly decreased time that is needed for the digestion of the wood to pulp. Many variations in the form of the apparatus may be resorted to without changing the process in any essential particular. While the apparatus is shown as mounted horizontally it is not confined in any sense to horizontal apparatus as vertical apparatus working on the same principles can be employed as well. Accordingly, it is to be understood that the invention is in no sense limited to the particular apparatus used but is directed to the process or method defined in the appended claims.

I claim:

1. The herein described process of producing cellulose fibres from wood or vegetable matter which consists in placing the said wood or vegetable constituents and chemicals in aqueous solution as commonly used for digestive purposes in a vessel, con-

tinuously cutting through the said constituents in an instantaneous rectilinear direction and continuously heating the digesting liquor and vegetable constituents contained within the said vessel.

2. The herein described process of producing cellulose fibres from wood or vegetable constituents and chemicals in aqueous solution as commonly used for digestive purposes in a vessel, cutting through the said constituents cylindrically in order to disintegrate the same and continually heating the digesting liquor and vegetable constituents contained within the said vessel or digestor.

In testimony whereof I affix my signature.

HERMAN B. KIPPER.

70

75

80

85

90

95

100

105

110

115

120

125

130